

Patented May 21, 1940

2,201,767

# UNITED STATES PATENT OFFICE

2,201,767

## LUBRICATING OIL

James A. Franceway, Jr., deceased, late of Madisonville, Ky., by James A. Franceway, Sr., administrator, Madisonville, Ky., and Garland H. B. Davis, Elizabeth, N. J., assignors to Standard Oil Development Company, a corporation of Delaware

No Drawing. Application July 2, 1936,  
Serial No. 88,612

26 Claims. (Cl. 87—9)

The present invention relates to the production of valuable lubricating oils, especially oils of low pour point and to methods for producing such products. This application is a continuation in part of our copending application Serial No. 623,814 filed July 21, 1932. Our invention will be fully understood from the following description of the products and their method of manufacture.

10 Lubricating oils obtained from petroleum and especially the higher grade lubricating oils contain waxy constituents and in consequence thereof are characterized by high pour points, that is to say, they become solid at relatively elevated temperatures, for example 30 or 40° F. or even 50 or 75° F., depending on the amount of wax present. It is the practice of refiners to remove a part or the whole of the wax so as to cause the oil to remain liquid to considerably lower temperatures, for example to 10° F. or even to 0° F. or lower, but this is an expensive operation and besides the wax is a desirable addition agent to the oil so that it is preferred not to remove it.

25 We have discovered a class of substances which when added to hydrocarbon oils improve their properties and when added to wax-containing oils even in small amounts cause the wax to crystallize in such a manner that the oil will remain fluid, and will pour at temperatures considerably below the normal pour points. These materials are also effective in decreasing the sludging tendencies of petroleum lubricating oils and in rendering such oils resistant to oxidation.

30 The substances which we have prepared are polymers of high molecular weight, soluble in oil and which do not undesirably affect the other properties of the oil. The polymers of a particular type produced in a special manner from 40 certain raw materials form the basis of the present invention.

35 The raw materials are contained in the general class of oxygenated organic materials which have relatively long straight hydrocarbon chains of, for example, 10 or 12 carbon atoms or more. They are preferably saturated. Oxygenated derivatives of the hydrocarbons contained in paraffin wax are desirable since they are characterized by substantially straight chains. The 45 normally liquid oils containing more than 10 or 12 carbon atoms per molecule are sometimes characterized by a marked branched and/or cyclic structure and if so are undesirable for the present purposes.

40 It is not, however, necessary that the chains of the oxygen-containing compounds be fully saturated. Olefins of more than 10 carbon atoms arranged in a relatively long straight chain are equally desirable.

45 These desirable polymers may be produced

from any compounds selected from the class of the alcohols, esters, ethers, acids, ketones and the like which contain hydrocarbon groups of at least 10 carbon atoms in substantially straight chains, and which contain, if any, preferably not 5 more than one carboxylic group. For example, stearic acid or its esters such as the methyl, ethyl or propyl stearates or oleic acid and its esters may be used; the alcohols above decyl, the corresponding aldehydes and ethers of such alcohols 10 and related substances such as the ketones are also available. While we prefer the naturally occurring acids or esters because of their cheapness, materials produced synthetically which may be mixtures of many different compounds, 15 or of compounds of the same type but of different number of carbon atoms, may be used with good results.

50 The method by which the above enumerated substances are treated to produce suitable polymers consists in the application thereto of high tension electric discharges. The process is carried out in the known manner under reduced pressure preferably below about 100 mm. absolute pressure but more elevated pressures about 20 to atmospheric, say 650 mm. may be used, and provision is made for continuously maintaining this reduced pressure. An alternating current of 60 cycles per second, for example, may be used but it is far more desirable to have greater 25 frequencies, say 10,000, 15,000 or even much higher. High voltages are also necessary, say 10,000 to 15,000 or higher, depending on the film of oil through which the current is to pass.

55 Any suitable apparatus as indicated above can 35 be used for our purpose, and many types are well known. The temperature of the material should be sufficient to keep it in a fluid state and it may be caused to flow in a thin film over the electrodes or, to splash, foam or squirt over them 40 in such a way as to subject the oil in thin films to the action of the high tension discharge. The electrodes may be placed in parallel, or in the form of plates which may be alternately dipped into and withdrawn from a bath of the 45 material or, they may be in the form of concentrically placed tubes or drums arranged in a horizontal direction and rocked about the horizontal axis through say 100 to 120 degrees or slowly rotated, and in this way the oily material 50 which may occupy something less than one-half of the annular space between the electrodes is washed up over the inner and the outer tube in such a way as to leave a film exposed to the current. If desired, a small amount of gas, for 55 instance nitrogen or hydrogen may be bubbled through the material undergoing treatment causing it to splash or foam. If desired, concentric electrodes may be used and rapidly rotated so as to cause the film of oil to form on 60

the outer electrode where it is thrown by centrifugal force.

In small scale equipment it has been found desirable to continuously add heat to the material either by jacketing the vessel or by withdrawing a portion of the material, heating it, and returning it to the vessel so as to maintain the wax or other solid material in a freely flowing liquid state. If the oil is naturally liquid ordinary temperatures are permissible, but even in that case slightly elevated temperatures from, say 100° to 500° F. or more, are desirable to keep the polymer in a state of reduced viscosity. In larger scale equipment where radiation losses are necessarily lower, less heat is required but it is ordinarily desirable in any case to provide thermostatic jackets so as to keep the conditions substantially the same during the treatment.

The polymers which we desire to form have molecular weights well in excess of 600 and substances as high as 1000 to 2000 and perhaps higher have been found in the product. The lower polymers apparently do not possess the desired pour depressing properties but it is extremely difficult to separate fractions closely and to state with exactitude at just what point this action begins. It may be stated, however, that unpolymerized fractions of the original material, for example alcohol may be removed from the heavier polymers by distillation and that the vaporized material generally possesses no pour inhibiting properties or, in any case, it is very weak and that the bottoms or residue concentrates the valuable or active material. The lighter fractions may be returned for retreatment in the same or in a successive treatment. The distillation should be conducted with fire and steam or with vacuum, and care should be taken to remove the lighter fractions without any substantial cracking of the residue.

While the oxygen-containing paraffinic material, by which we mean material containing relatively long hydrocarbon chains and oxygen, may be used along, it is permissible to add there-to a substance of a cyclic structure such as benzol or naphthalene, their hydrogenated or alkylated derivatives such as toluol, xylol and ethyl naphthalene. Hydroxylated aromatics, such as the phenols and naphthols, may be used for this purpose, as well as the nitrated aromatics or the amino derivatives of the type of aniline, naphthylamine and the like. Even cyclic terpenes may be used. These materials are added in proportion of, say 10 to 14 or 20% of the paraffinic material and the condensation takes place in substantially the same manner as indicated above, but it is clear that the aromatic or cyclic material actually takes part in the combination.

The time of treatment varies according to the power input and consequently if that is low a time of say 100 or 150 hours may be required, whereas if it is higher the work may be accomplished in 50 or 25 hours or even in less time. The amount of material to be used for our purposes may be generally described as in pour inhibiting proportions. If too much of the material is used the pour inhibiting effect tends to diminish so that there is a decided optimum for pour depressing. The actual amount to be used, of course, also depends on the concentration of the active substance in the oily polymers. Ordinarily, if a good grade of polymer is produced 1% is sufficient, but in some instances as little as .1 to .5% may be sufficient, and in other cases 2 to 5% may be required. It is desirable, as in-

dicated above, to concentrate the inhibitor to some extent and this is preferably done by distilling off the lower readily distillable fractions, for example, by vacuum distillation or by other suitable means. Where the agent is well concentrated the pour inhibiting effect may be obtained without substantial increase in viscosity.

The polymers also serve to stabilize lubricating oils against oxidation and development of sludge. They are effective as oxidation inhibitors and sludge preventers in oils which contain little or no wax, as well as in waxy oils. They are effective for these purposes in concentrations of about 0.1% to 5 or 10% and may be used in even larger amounts, ordinarily 1 or 2% will be found satisfactory.

The following examples are presented to illustrate suitable methods for the preparation of the herein described products, and their use in lubricating oil blends.

*Example 1.*—An alcohol fraction was prepared by oxidizing at a low temperature a paraffin wax derived from petroleum. Non-acidic oxygen containing components were separated from the saponified oxidation product and from the un-oxidized hydrocarbons by extraction first with naphtha and then with aqueous methanol. The alcohol extract was distilled under vacuum at an absolute pressure of 20 mm. of mercury, the 0-56% cut being recovered as distillate. This distillate of crude alcohols was hydrogenated to convert the ketones therein to alcohols. The hydrogenated alcohol fraction was then subjected to silent electric discharge of an alternating current of 1200 cycles at 7000 volts at a pressure of about 4 cm. of mercury. Hydrogen was passed through the oil throughout the test to promote foaming. By this means the alcohol fraction was raised from an initial viscosity of 43 seconds Saybolt at 210° F. to a viscosity of 575 seconds Saybolt at 210° F., and from an initial average molecular weight of 304 to an average molecular weight of about 1060.

Blends of this material in concentrations of 2% were prepared with highly refined petroleum lubricating oils and it was observed that both the sludging tendency of the oils and their susceptibility to oxidation were substantially decreased. Results of tests on the original oils and the blends are presented in the following table:

| Lubricating oil             | Sludge (Sligh test) | Oxidation rate cc. 0/10 gm. Oil/15 min. |
|-----------------------------|---------------------|-----------------------------------------|
| A. (65 vis/210° F.)         | 1.3                 | 103, 108, 67, 59                        |
| A. +2% voltolized alcohols  | 0.5                 | 55, 72, 53, 42                          |
| B. (46 vis/210° F.)         | 13.4                | 82, 92, 71, 51                          |
| B. +2% unvoltolized alcohol | 11.1                | 80, 105, 72, 51                         |
| B. +2% voltolized alcohol   | 1.1                 | 50, 44, 49, 51                          |

*Example 2.*—Cetyl alcohol was thickened by subjection to silent electric discharge until a voltolized product having a viscosity of 600 seconds Saybolt at 210° F. was obtained. 2% of this voltolized cetyl alcohol was added to a petroleum lubricating oil having a Sligh number of 12. The Sligh number of the resulting blend was 0.8, thereby indicating a very substantial reduction in the sludging tendency of the oil. Voltolized stearyl alcohol and voltolized lauryl alcohol gave comparable reductions in the Sligh number of the lubricating oil.

The tendency of a lubricating oil to form separable sludge is determined by the Sligh test which involves exposing a sample of the oil to the action of oxygen at 392° F. The Sligh test is de-

scribed in Proc. A. S. T. M., vol. 24, 964 II (1924). The Sligh number of an oil is the number of milligrams of sludge deposited by 10 cc. of the oil when treated at the temperature specified for a given time with a given quantity of oxygen.

The susceptibility of a lubricating oil to oxidation at motor operating temperatures is determined by measuring the amount of oxygen that a given sample of the oil will absorb in a given time at a given temperature when blown with oxygen at a given rate. This test as conducted in the above examples is a determination of the number of cc.'s of oxygen absorbed by 10 gm. of the oil per 15 minute interval of exposure at 15 392° F.

While it is preferred to electrically treat the raw material in a substantially concentrated state, it can be polymerized while dissolved in a suitable oil stock such as a lubricating oil or 20 a hydrogenated lubricating oil. The oil may also contain substantial amounts of wax. The oil in such case is polymerized to some extent as will be appreciated, and even though the product may be rich in wax, it still has a low pour point due 25 to the presence of the inhibitor produced in situ. This product can be used as an inhibitor and added to other oils such as natural waxy oils or to hydrogenated or synthetic oils, or may be used as a lubricant as such.

30 Our invention is not to be limited by any theory of the mechanism of electrical condensation, nor of pour reduction, but only to the following claims in which we wish to claim all novelty inherent in the invention.

We claim:

1. A process for producing polymers of high molecular weight and soluble in lubricating oils, comprising subjecting substantially saturated oxygen-containing material characterized by a relatively long straight hydrocarbon chain and containing not more than one carboxylic group to a high tension electric discharge for a period sufficient to effect substantial polymerization.

2. A process according to claim 1, in which the said hydrocarbon chain contains at least 10 carbon atoms.

3. A process according to claim 1, in which the said material comprises a fatty acid of at least 10 carbon atoms.

4. A process according to claim 1, in which the said material comprises an ester having a straight hydrocarbon chain of at least 10 carbon atoms.

5. An improved process for producing polymeric alcohols, comprising subjecting an alcohol to a high tension electric discharge for a period sufficient to effect substantial polymerization.

6. An improved process for producing polymeric alcohols, comprising subjecting an alcohol in liquid condition to high frequency, high tension electric discharge until substantial polymerization is effected.

7. An improved process for producing polymeric alcohols, comprising subjecting higher alcohols having more than 10 carbon atoms while in liquid condition to high frequency, high tension electric discharge while under reduced pressure and at temperatures below about 500° F. for a period of time to effect substantial polymerization.

70 8. A process for producing polymers according to claim 1, in which a cyclic compound is subjected to the electric discharge with the said oxygen-containing material.

9. A process according to claim 6, in which the alcohol is polymerized along with a compound of cyclic structure.

10. A process according to claim 7, in which the alcohol is polymerized along with an aromatic 5 hydrocarbon.

11. An organic polymer produced according to the process of claim 1.

12. A polymeric acid prepared by subjecting an unpolymerized substantially saturated fatty 10 acid of at least 10 carbon atoms to silent electric discharge for a prolonged period.

13. A polymeric ester prepared by subjecting an unpolymerized ester having a straight carbon chain of at least 10 carbon atoms and having not 15 more than one carboxylic group to silent electric discharge for a prolonged period.

14. A polymeric alcohol prepared by subjecting an unpolymerized alcohol to silent electric 20 discharge for a prolonged period. 20

15. A polymeric alcohol prepared by subjecting an unpolymerized alcohol having at least 10 carbon atoms to the action of a silent electric discharge for a prolonged period.

16. A polymer of high molecular weight, soluble in lubricating oils, produced by subjecting a mixture of a compound of cyclic structure and an oxygen-containing material characterized by a relatively long straight hydrocarbon chain and containing not more than one carboxylic group, 25 to the action of a silent electric discharge for a prolonged period.

17. A composition according to claim 14, in which the alcohol is polymerized with a compound of cyclic structure. 35

18. A composition of matter comprising a mineral lubricating oil and a polymeric material produced according to the process of claim 1.

19. A composition of matter comprising a mineral lubricating oil and a polymeric material 40 described in claim 16.

20. A composition of matter comprising a mineral lubricating oil and polymeric alcohol prepared by subjecting an unpolymerized alcohol to the action of a high tension electric discharge for a time sufficient to effect polymerization.

21. A composition of matter comprising a mineral lubricating oil and a polymeric alcohol prepared by subjecting unpolymerized alcohol in the presence of a compound of cyclic structure, to the action of a high tension electric discharge for a time sufficient to effect polymerization.

22. A composition of matter comprising a mineral lubricating oil and a polymeric alcohol prepared by subjecting an unpolymerized alcohol containing at least 10 carbon atoms with a material of cyclic structure to the action of a high tension electric discharge for a time sufficient to effect polymerization.

23. Process according to claim 1 in which the said material contains no halogen and comprises a fatty acid of at least 10 carbon atoms.

24. A polymeric acid according to claim 12 and containing no halogen.

25. A polymer according to claim 16 in which the compound of cyclic structure is a phenol.

26. A polymer according to claim 16 in which the compound of cyclic structure is naphthalene.

JAMES A. FRANCEWAY, SR.,  
Administrator of Estate of James A. Franceway,  
Jr., Deceased.

GARLAND H. B. DAVIS.